

## UNITED STATES PATENT OFFICE

GEORGE BRAY, OF LEEDS, ENGLAND, ASSIGNOR TO GEO. BRAY & COMPANY LIMITED,  
OF LEEDS, ENGLAND

ELECTRICAL HEATING ELEMENT

No Drawing. Application filed January 28, 1931, Serial No. 511,910, and in Great Britain February 8, 1930.

This invention relates to electrical heating elements of the type comprising a resistor enveloped in a mass of refractory material enclosed within a shallow sheet metal casing 5 or sheathing.

The sheet metal casing or sheathing has been made of a chrome iron or steel but it is found that if there is a high percentage of chromium which will cause the metal to resist oxidation the emission of heat therefrom is lessened and the object of the invention is to provide a case or sheathing of non-oxidizable chrome metal with a surface that will quickly and readily dissipate or emit the heat 15 generated in the interior of the heating element.

According to the invention the metal case or sheathing of the heating element is made from a chrome iron or steel having a high 20 percentage of chromium to render it non-oxidizable the surface being coated with a fine coating or layer of heat emitting material such as copper or iron oxidized by the application of heat.

25 The metal case or sheathing may be of known construction or of the construction described in my application Number 511,909, filed concurrently herewith.

It is made of a chrome iron or steel having 30 about 20% of chromium to render it non-oxidizable with or without nickel. The surface preferably after the case is constructed is coated by plating or spraying with a layer of copper and is subsequently heated to a 35 degree sufficient to oxidize the surface of copper (say 600° to 700° C.).

The invention may be applied to elements either annular, straight or flat.

40 What I claim as my invention and desire to protect by Letters Patent is:—

1. An electric heating element of the type referred to constructed with a sheathing of highly resisting non-oxidizable chrome metal the exterior surface of which is coated with 45 a fine layer of metallic oxide.

2. An electric heating element of the type referred to constructed with a case of highly resisting non-oxidizable chrome metal the exterior surface of which is coated with a 50 fine layer of copper oxide.

3. A metal case for an electric heating element constructed of non-oxidizable chrome metal in combination with a fine layer of metal oxidized thereon.

4. A sheathing for an electric heating element constructed of highly resisting nickel chrome coated with a fine layer of copper oxidized thereon.

In testimony whereof I have hereunto set my hand this 9th day of January 1931.

GEORGE BRAY.

65

70

75

80

85

90

95

100